

## UNITED STATES PATENT OFFICE

2,220,805

## TREATMENT FOR ANIMAL FIBER

William Beach Pratt, Boston, Mass.; Annette Harris Pratt, administratrix of said William Beach Pratt, deceased; assignor to Aldox Corporation, Dover, Del., a corporation of Delaware

No Drawing. Application July 18, 1938,  
Serial No. 219,823

3 Claims. (Cl. 8—128)

My invention is an improved treatment for animal or nitrogenous fibers, such as wool, hair and silk.

Such treatment involves essentially the attachment of an aldehyde radical to the molecular structure of the fiber and the substitution of water for the aldehyde radical by the oxidation of the latter in the presence of water.

The attachment of the aldehyde radical to the nitrogenous fiber must be carried out in the absence of substances having a greater affinity for the aldehyde present than the affinity for the nitrogenous fiber thereof, and is preferably effected in an aqueous bath free from substances reacting with aldehyde to form condensation products. The subsequent oxidation of the aldehyde radical should also be carried out in the absence of any substantial alkalizing influence.

The fibers are preferably treated in accordance with my invention before being subjected to ordinary cleansing treatments which so deteriorate or break down the fibers that their natural characteristics cannot be restored. My treatment is applicable to the fibers before or after removal from the skins or in the form of fibers, per se, filaments, yarns or fabrics.

By my method of treatment, not only is a chemical compound formed between the aldehyde and fiber molecules, but the greasy, gummy, waxy, oily, and ceresin substances naturally present in animal fibers have their melting points lowered and their solubility and emulsibility increased by the action of aldehyde thereon, particularly in the presence of suitable penetrants and detergents.

The lowering of the melting points of the greases, waxes, etc., is accompanied by an increase in the resistivity of the fiber itself to the action of heat, hence the treatment may be carried out at a temperature such that the oils, greases and waxes are rapidly emulsified without injury to the fiber itself.

The removal of such substances and the subsequent removal of the aldehyde radical gives the fibers a lofty hand and permanent set, makes possible the bleaching of such fibers without deteriorating effects, renders the fibers more resistant to the physical effects resulting from washing untreated fibers in alkaline solutions, makes the fibers more hygroscopic, and improves dye absorption and the tintorial effect of dyes on the fibers.

My treatment is carried on preferably under atmospheric pressure. While the temperature should be sufficiently high for the ready emulsifi-

cation with water of the softened, greasy, gummy and like constituents, it should not be sufficiently high to impair the natural elasticity of the fiber or to cause wasteful loss of aldehyde from aqueous solution. The loss of aldehyde from aqueous solution may be retarded by forming in the bath a loose bed of fibers of substantial thickness.

The attachment of the aldehyde to the molecules of the fiber appears to take place most readily when the bath is substantially neutral, or has a pH of say 7 to 9 and free from any substance reactive with aldehyde to form a condensation product. The fiber may have the aldehyde combined therewith by immersion in a bath, of such pH, containing initially only trioxymethylene. After sufficient aldehyde has been released from the trioxymethylene and attached to the fiber, suitable detergents, such as neutral soap and borax, may be added to the bath to facilitate emulsification and removal of the grease and waxes. A good attachment of the aldehyde to the fiber, and a somewhat more rapid processing is, however, secured when the detergents are added to the bath at the beginning of the aldehyde treatment, since the aldehyde and borax both tend to reduce the pH which would result from the soap alone. If a soap producing a pH of, say, 10.2 is used, sufficient borax and aldehyde may be used to reduce the pH of the bath to around 8.

Any tendency toward decomposition of the soap is avoided by the maintenance of a temperature below its decomposition point and counteracted by the inclusion of the borax in the bath. The action of borax in keeping the solution at a pH value as low as possible without injuring the properties of the detergent, is of distinct advantage in the treatment of animal fiber.

I may provide the bath for giving the aldehyde treatment by diluting with water standard commercial aqueous solution of formaldehyde of say 37° to 40° concentration, or I may employ reversible polymerization products of formaldehyde free from extraneous substances. Such products as trioxymethylene or para-formaldehyde may be employed. Where commercial formaldehyde solutions are used, the solubility or dilution is uniformly distributed through such solution regardless of the water temperature, but when para-formaldehyde or trioxymethylene is employed the temperature must be raised to at least 120° F. to insure complete solubility throughout the aqueous solution of formaldehyde produced by the splitting up of these polymerization products. But even when a dilute commercial solu-

tion of formaldehyde is employed, the bath should be maintained at a temperature of at least 120° F. in order that the free formaldehyde gas present in the solution may adequately act on the 5 greases and gums and combine with the keratin or fibroin on the fiber.

The neutral soap, borax and aldehyde, in the form of trioxymethylene, may be well mixed together in dry form and then dissolved in the 10 water to form a bath substantially free from substances with which aldehyde tends to form condensation products or for which it has a greater affinity than it has for the animal fiber. The bath should have a temperature which 15 effects the liberation of the aldehyde and the chemical combination thereof with the molecular structure of the animal fiber and increase the solubility and factors of emulsification of the greasy and gummy constituents of the fiber. 20 As the aldehyde lowers the melting points of the greasy and gummy constituents and increases the resistance of the fiber to the action of heat, the treatment can be readily carried on at a temperature of say 140° F. which is above 25 the point to which the aldehyde lowers the melting point of the gummy and greasy constituents and well below a point injurious to the aldehyde treated fibers.

The aldehyde so combines with the molecules 30 of the fiber as to resist removal by repeated washings, which washings effect the substantially complete removal of the foreign matter such as grease, lanolin, seresin, and other oily and gummy substances.

35 After the washing of the fibers, the aldehyde radical or constituent of the keratinous or fibroin molecules is removed by the oxidation thereof into an acid in the presence of water, which takes the place of the aldehyde radical and hydrates 40 the fibers.

The removal of the aldehyde radical should preferably be effected by means of an oxidizing agent capable of the use in neutral or slightly acid solutions as it is desirable that the oxidation 45 be carried on under conditions free from alkalinizing influences.

I have successfully employed a solution containing, say, 0.25% of potassium permanganate (based on the weight of the fiber) and a small 50 amount of sulphuric acid or magnesium sulphate to act as a buffer in neutralizing any caustic soda that might be freed through reaction. Other suitable oxidizers for removing the aldehyde after it has been firmly attached to the 55 fiber molecules and effecting substitution of water for the aldehyde are hydrogen peroxide solution, sodium dioxide solution, and sodium perborate solution.

By such treatment not only are sheared wools 60 clarified and freed from grease, oil and stains and given a lofty feel, but even pulled wool so treated is so improved as to be indistinguishable from sheared wool.

The following is a specific example, but by 65 way of illustration only, of the carrying out of my invention for the treatment of wool.

A mixture of say 40 pounds of trioxymethylene, 20 pounds of borax, and 100 pounds of neutral 70 soap of low titer, is dissolved in water sufficient in amount for the wetting and immersion of say ten thousand pounds of wool. The treatment may be carried on in the standard equipment commonly used for wool scouring, but the treating tanks should preferably be made of 75 wood and be substantially free from any ex-

posed iron. The treatment may be carried on either in batch or continuously, depending upon the character of the equipment employed.

The wool is subjected to the action of the solution at a temperature between 120° F. and 140° F. and preferably in the neighborhood of 130° F. for approximately fifteen minutes. At the end of this time the wool is passed through a washing tank where the impurities, soap and any uncombined aldehyde are thoroughly removed from the fiber. The presence of the combined aldehyde in the fiber may be tested by treatment of a washed sample with Fehling's solution. When the aldehyde bath is initially free of detergents, a somewhat longer combining time is generally desirable than where detergents are initially present.

The thoroughly cleaned wool is then passed through an aqueous solution containing say 0.25% of potassium permanganate or sodium permanganate, based on the weight of the wool, and at a temperature preferably between 104° F. and 120° F. The aldehyde treated fiber acts promptly to reduce the permanganate solution to a clear aqueous solution with the permanganate salts of decomposition precipitated in or upon the animal fiber. This precipitation will ordinarily take place in about ten minutes. When the precipitation is complete, the fibers are passed directly into a solution of sodium bisulphite and/or sulphurous acid to remove the decomposition products from the reduction of permanganate. The wool is then rinsed in running water to wash out the soluble products so formed. In regular commercial practice, and where it is not necessary to secure the highest degree of whiteness, a regular hydrogen peroxide bleach may be employed, or any standard method for bleaching the wool as is practiced after the usual scouring operation.

The oxidizing treatment may be so limited as to merely free the animal fiber from the aldehyde radical to hydrate the fiber and permit subsequent bleaching, or the oxidation may be carried on until the fiber is partially bleached or bleached 45 to a pure white.

I have heretofore pointed out in my co-pending application for Patent 2,126,809, whereof the present application is a continuation in part, that nitrogenous fibers having a sulphur containing radical may be advantageously treated with aldehyde to improve the texture and loftiness of the fibers and with oxidizing agents to prevent the formation of condensation products from the aldehydic constituent and effect bleaching of the fiber. Such aldehydic and oxidizing treatments of certain fibers are best effected after subjecting the fibers to an ammoniacal treatment which attacks the sulphur constituent of the sulphur radical of the fiber, to the ultimate removal or rearrangement of the sulphur radical. Such ammoniacal treatment renders the fiber much more readily susceptible to the action of the aldehydic and oxidizing agents. By such ammoniacal, aldehydic, and oxidizing treatments, naturally black fibers, such as wool, hair, or mohair, alpaca or fur, may be bleached to a pure white.

In the treatment of such fibers, or of fabrics or 70 yarns composed of or containing them, they may be immersed in and drawn through an aqueous solution containing approximately 6% of ammonia, approximately 1% of aldehyde, 1% of neutral soap, and 1% of sodium perborate or other suitable oxidizing agents based on the 75

weight of the fiber and contained in an open vessel or jig.

I have found that commercial soaps may be effectively neutralized by redrying them in the presence of carbon dioxide and thereby render it suitable for use in conjunction with the aldehydic treatment without danger of forming condensation products.

After immersion for approximately two hours 10 at a temperature of from 130° to 140°, the fibers are rendered lofty, white and free from grease and dirt. Should the fabrics be darkly pigmented naturally, a larger percentage of oxidizing agent may be used or the fibers may be given repeated 15 treatments until a pure white is obtained.

For degumming and bleaching silk the same treatment may be used, but the ammonia should be dispensed with.

Howsoever the practice of my invention is carried on, the baths employed should contain no reagents free to combine with aldehyde to form condensation products or deleteriously effect the nitrogenous fibers, as, for instance, soda ash, caustic soda, trisodium phosphate or sodium bisulphate. The use of soaps that tend to break down readily and release alkali at the treatment temperatures should be avoided. The presence in a bath containing aldehyde of reagents free to combine therewith to form insoluble condensation products not only retards or prevents the liberation of free aldehyde gas and the combining thereof with the molecules of the animal fiber, but may also stain the goods and even effect removal of some aldehyde radicals which have been attached to the fiber molecule. The formation of objectionable condensation products from the reaction of the aldehyde with such reagents will frequently take place at lower temperatures than the temperature at which aldehyde satisfactorily combines with molecules of animal fiber. Hence 40 while such condensation products of aldehyde and alkali may have uses under other conditions, such condensation products are distinctly inimical to the practice of the present invention.

The reaction of the aldehyde on the greases and gums inherent in natural animal fibers appears to be both chemical and physical. Their melting points are lowered and they appear to change in surface tension to increase water absorption. They are rendered by my treatment readily removable from the animal fiber by washing, particularly when proper detergents or emulsifying agents are employed in a subsequent washing operation.

Having described my invention, I claim:

1. In the treatment of animal fibers having a greasy or gummy constituent, the steps which include lowering the melting point of such constituent by treatment with an aldehyde in the presence of a detergent of the group consisting of a neutral soap and borax at a temperature below the decomposition point of the detergent and above the point to which the aldehyde lowers the melting point of the constituent.

2. In the treatment of animal fibers having a greasy or gummy constituent, the steps which include treating the fibers with an aqueous solution containing a detergent of the group consisting of a neutral soap and borax and a reversible polymerization product of formaldehyde free from extraneous substances at a temperature at which the melting point of such constituent is lowered and aldehyde combines with the molecules of the fiber.

3. In the treatment of keratinous fiber having a natural gummy or greasy constituent, the steps which include impregnating the fibers in an aqueous formaldehyde neutral soap borax solution devoid of reagents combining with formaldehyde in the presence of borax and at a temperature substantially in the range of 120 to 140° F. until the melting point of such constituent is lowered and an aldehyde radical has formed on the fiber, and substituting water for the aldehyde radical by oxidizing the aldehyde to acid in the presence of water prior to any reaction of the radical to form a condensation product.

WILLIAM BEACH PRATT.